

## UNITED STATES PATENT OFFICE.

KARL HEINRICH WOLMAN, OF BERLIN-GRUNEWALD, GERMANY.

## WOOD-PRESERVING MEANS.

No Drawing. Application filed November 9, 1923, Serial No. 673,850, and in Germany September 25, 1923.

My invention relates to a new and improved wood preserving composition which is suited to protect permanently the wood from the attacks of wood-destroying fungi and animals. The invention is based on the observation that the wood preserving composition disclosed in the following lines possesses a by far greater antiseptic effect than it could be expected according to the effect 5 of the unmixed components of which said composition consists. The new wood preserving means consists principally of nitrated cresols, fluorine compounds and arsenic compounds which are soluble in water 10 and apt to counteract the action of fungi, and, finally, of such substances which are apt to protect iron from being affected by solutions of the said wood preserving means.

It has been found that in a thus composed 20 wood preserving composition the preserving properties of the individual component substances do not simply sum up but that the effect of the preserving means composed in the manner hereinafter described is considerably greater than the summed effect of the 25 individual unmixed substances composing it. The preserving composition in question is able to protect the wood treated therewith from the attack of wood-destroying fungi, 30 as well as from the attack of animals, especially insects. It is very difficult to lixiviate it out of the wood, it is chemically not easily changeable and may be used for the impregnation of the wood in any desired manner and 35 with any desired apparatus.

The nitrated cresols may be mononitrocresols or dinitro-cresols. Also the compounds of the nitrated cresols with organic bases have delivered good results. As fluorine compound every stable, water-soluble fluor-salt, for instance sodium silico-fluoride or fluoride of sodium, may be used. As arsenic compounds preferably salts are used

which are chemically stable and very poisonous for fungi and animals. Thus, for instance, arsenic acid or the salts thereof may be employed. As protective means for iron alkali metal chromates or bichromates may be used.

Example: 10 parts of o-dinitro-cresol, 40 45 parts of fluoride of sodium, 30 parts of arsenate of sodium, and 20 parts of bichromate of sodium, are mixed with each other. This mixture is, preferably, dissolved in water, in such a proportion that a 2%-solution is 50 obtained, which is used for impregnating the 55 wood.

The new wood preserving composition may be used in connection with other compounds of antiseptic effect or those adapted to diminish the inflammability of the wood. Impregnating the wood therewith may be effected in any desired manner, for instance in open wooden troughs, or in troughs of cement, or in iron containers, may be in connection either with reduced or increased pressure, or by boiling the wood in the respective solution, and so on.

Concerning the addition of an iron-protective means I point out that this addition 70 is necessary from the reason as otherwise the iron receptacles, troughs, or the like, in which the wood is impregnated would be affected by the wood preserving composition introduced into said receptacles, etc. This is true especially of the nitrated phenols and the salts thereof which have the property of affecting iron like acids. From this reason bichromate of sodium or an equivalent substance is added 75 to the composition.

I claim:

A wood preserving composition consisting of dinitro-cresol, sodium fluoride, salts of arsenic acid, and bichromates of alkalies.

In testimony whereof I affix my signature.

KARL HEINRICH WOLMAN.